



US011441205B2

(12) **United States Patent**  
**Oh et al.**

(10) **Patent No.:** **US 11,441,205 B2**  
(b4) **Date of Patent:** **Sep. 13, 2022**

(54) **COLD-ROLLED STEEL PLATE FOR HOT FORMING, HAVING EXCELLENT CORROSION-RESISTANCE AND SPOT-WELDABILITY, HOT-FORMED MEMBER, AND METHOD FOR MANUFACTURING SAME**

(71) Applicant: **POSCO**, Pohang-si (KR)

(72) Inventors: **Jin-Keun Oh**, Gwangyang-si (KR); **Yeol-Rae Cho**, Gwangyang-si (KR); **A-Ra Cho**, Incheon (KR); **Jin-Ho Cha**, Gwangyang-si (KR); **Si-Myoung Heo**, Gwangyang-si (KR); **Jeong-Won Seo**, Gwangyang-si (KR); **Seong-Woo Kim**, Gwangyang-si (KR)

(73) Assignee: **POSCO**, Pohang-si (KR)

(\*) Notice: Subject to any disclaimer, the term of this patent is extended or adjusted under 35 U.S.C. 154(b) by 723 days.

(21) Appl. No.: **16/336,645**

(22) PCT Filed: **Sep. 26, 2017**

(86) PCT No.: **PCT/KR2017/010639**

§ 371 (c)(1),  
(2) Date: **Mar. 26, 2019**

(87) PCT Pub. No.: **WO2018/056792**

PCT Pub. Date: **Mar. 29, 2018**

(65) **Prior Publication Data**

US 2020/0385833 A1 Dec. 10, 2020

(30) **Foreign Application Priority Data**

Sep. 26, 2016 (KR) ..... 10-2016-0123273

(51) **Int. Cl.**

**C21D 9/46** (2006.01)  
**B21B 3/02** (2006.01)

(Continued)

(52) **U.S. Cl.**  
CPC ..... **C21D 9/46** (2013.01); **B21B 3/02** (2013.01); **B21D 22/022** (2013.01); **C21D 6/004** (2013.01);

(Continued)

(58) **Field of Classification Search**  
None  
See application file for complete search history.

(56) **References Cited**

**U.S. PATENT DOCUMENTS**

6,296,805 B1 10/2001 Laurent et al.  
10,590,503 B2 \* 3/2020 Hasegawa ..... C21D 8/0236  
(Continued)

**FOREIGN PATENT DOCUMENTS**

CN 102666923 9/2012  
CN 105814227 7/2016  
(Continued)

**OTHER PUBLICATIONS**

International Search Report—PCT/KR2017/010639 dated Jan. 16, 2018.

(Continued)

*Primary Examiner* — Daniel J. Schleis

(74) *Attorney, Agent, or Firm* — Cantor Colburn LLP

(57) **ABSTRACT**

Provided is a cold-rolled steel plate for hot forming, which is excellent in corrosion-resistance and spot-weldability, contains, by weight %, C: 0.1-0.4%, Si: 0.5-2.0%, Mn: 0.01-4.0%, Al: 0.001-0.4%, P: 0.001-0.05%, S: 0.0001-0.02%, Cr: 0.5% to less than 3.0%, N: 0.001-0.02%, and a balance of Fe and inevitable impurities, satisfying formula (1) below, and includes an Si amorphous oxidation layer continuously or discontinuously formed at a thickness of 1 nm-100 nm on the surface thereof. Formula (1):  $1.4 \leq 0.4\text{Cr} + \text{Si} \leq 3.2$  (wherein element symbols denote measurements of respective element contents by weight %).

**4 Claims, 5 Drawing Sheets**



| (51) Int. Cl. |                   | FOREIGN PATENT DOCUMENTS                                                                                                                                                                                                                                                                                                                                                                                                                                                                                                                                                                                        |    |                       |
|---------------|-------------------|-----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|----|-----------------------|
|               | <i>B21D 22/02</i> | (2006.01)                                                                                                                                                                                                                                                                                                                                                                                                                                                                                                                                                                                                       | EP | 2684972 1/2014        |
|               | <i>C21D 6/00</i>  | (2006.01)                                                                                                                                                                                                                                                                                                                                                                                                                                                                                                                                                                                                       | EP | 3020842 5/2016        |
|               | <i>C21D 8/02</i>  | (2006.01)                                                                                                                                                                                                                                                                                                                                                                                                                                                                                                                                                                                                       | EP | 3054025 8/2016        |
|               | <i>C22C 38/00</i> | (2006.01)                                                                                                                                                                                                                                                                                                                                                                                                                                                                                                                                                                                                       | JP | 61110757 5/1986       |
|               | <i>C22C 38/02</i> | (2006.01)                                                                                                                                                                                                                                                                                                                                                                                                                                                                                                                                                                                                       | JP | 2005133180 5/2005     |
|               | <i>C22C 38/04</i> | (2006.01)                                                                                                                                                                                                                                                                                                                                                                                                                                                                                                                                                                                                       | JP | 2007113108 5/2007     |
|               | <i>C22C 38/06</i> | (2006.01)                                                                                                                                                                                                                                                                                                                                                                                                                                                                                                                                                                                                       | JP | 2014508854 4/2014     |
|               | <i>C22C 38/20</i> | (2006.01)                                                                                                                                                                                                                                                                                                                                                                                                                                                                                                                                                                                                       | KR | 20090124263 12/2009   |
|               | <i>C22C 38/22</i> | (2006.01)                                                                                                                                                                                                                                                                                                                                                                                                                                                                                                                                                                                                       | KR | 20110065949 6/2011    |
|               | <i>C22C 38/24</i> | (2006.01)                                                                                                                                                                                                                                                                                                                                                                                                                                                                                                                                                                                                       | KR | 20130076959 7/2013    |
|               | <i>C22C 38/26</i> | (2006.01)                                                                                                                                                                                                                                                                                                                                                                                                                                                                                                                                                                                                       | KR | 20140002272 1/2014    |
|               | <i>C22C 38/50</i> | (2006.01)                                                                                                                                                                                                                                                                                                                                                                                                                                                                                                                                                                                                       | KR | 20140138801 12/2014   |
|               | <i>C22C 38/54</i> | (2006.01)                                                                                                                                                                                                                                                                                                                                                                                                                                                                                                                                                                                                       | KR | 20150053625 5/2015    |
| (52)          | <b>U.S. Cl.</b>   |                                                                                                                                                                                                                                                                                                                                                                                                                                                                                                                                                                                                                 | KR | 20160077582 7/2016    |
|               | CPC .....         | <i>C21D 6/005</i> (2013.01); <i>C21D 6/008</i> (2013.01); <i>C21D 8/0205</i> (2013.01); <i>C21D 8/0226</i> (2013.01); <i>C21D 8/0236</i> (2013.01); <i>C21D 8/0247</i> (2013.01); <i>C22C 38/001</i> (2013.01); <i>C22C 38/002</i> (2013.01); <i>C22C 38/008</i> (2013.01); <i>C22C 38/02</i> (2013.01); <i>C22C 38/04</i> (2013.01); <i>C22C 38/06</i> (2013.01); <i>C22C 38/20</i> (2013.01); <i>C22C 38/22</i> (2013.01); <i>C22C 38/24</i> (2013.01); <i>C22C 38/26</i> (2013.01); <i>C22C 38/50</i> (2013.01); <i>C22C 38/54</i> (2013.01); <i>C21D 2211/003</i> (2013.01); <i>C21D 2211/005</i> (2013.01) | WO | 2009145563 12/2009    |
|               |                   |                                                                                                                                                                                                                                                                                                                                                                                                                                                                                                                                                                                                                 | WO | WO2009145563 * 3/2010 |
|               |                   |                                                                                                                                                                                                                                                                                                                                                                                                                                                                                                                                                                                                                 | WO | 2013047836 4/2013     |
|               |                   |                                                                                                                                                                                                                                                                                                                                                                                                                                                                                                                                                                                                                 | WO | 2014166630 10/2014    |
|               |                   |                                                                                                                                                                                                                                                                                                                                                                                                                                                                                                                                                                                                                 | WO | 2015093043 6/2015     |
|               |                   |                                                                                                                                                                                                                                                                                                                                                                                                                                                                                                                                                                                                                 | WO | 2016093598 6/2016     |

(56) **References Cited**

## U.S. PATENT DOCUMENTS

|                 |         |                 |
|-----------------|---------|-----------------|
| 2008/0053580 A1 | 3/2008  | Drillet et al.  |
| 2012/0325376 A1 | 12/2012 | Makimizu et al. |
| 2013/0295402 A1 | 11/2013 | Oh et al.       |
| 2014/0234658 A1 | 8/2014  | Nozaki et al.   |
| 2015/0020992 A1 | 1/2015  | Shottler et al. |
| 2016/0319385 A1 | 11/2016 | Hasegawa et al. |
| 2017/0369974 A1 | 12/2017 | Kim et al.      |

## OTHER PUBLICATIONS

Chinese Office Action—Chinese Application No. 201780059276.9 dated Apr. 27, 2020, citing WO 2009/145563, CN 105814227, KR 2016-0077582, KR 2016-0078851, JP 2007-113108, KR 2013-0076959, and CN 102666923.

Japanese Office Action—Japanese Application No. 2019-515875 dated Mar. 24, 2020, citing JP 2014-508854, JP S61-110757, WO 2013/047836, KR 10-2009-0124263, KR 10-2016-0078851, JP 2007-113108, WO 2015/093043, and KR 10-2013-0076959.

European Search Report—European Application No. 17853506.8, dated Aug. 2, 2019, citing WO 2009/145563, EP 3 054 025, KR 2013 0076959, KR 2016 0077582, WO 2016/093598, EP 2 684 972, US 2008/053580, EP 3 020 842 and WO 2014/166630.

\* cited by examiner

FIG. 1



FIG. 2



FIG. 3



FIG. 4



FIG. 5



FIG. 6



FIG. 7



**COLD-ROLLED STEEL PLATE FOR HOT FORMING, HAVING EXCELLENT CORROSION-RESISTANCE AND SPOT-WELDABILITY, HOT-FORMED MEMBER, AND METHOD FOR MANUFACTURING SAME**

TECHNICAL FIELD

The present disclosure relates to a cold-rolled steel plate for hot forming, having excellent corrosion-resistance and spot-weldability, a hot-formed member, and a method for manufacturing the same.

BACKGROUND ART

Members manufactured through a hot-forming process have been increasingly applied to use as structural members of vehicles to improve fuel efficiency by reducing a weight of a vehicle and to improve crashworthiness by achieving ultra-high strength, and a large amount of research has accordingly been conducted.

A representative technique is the invention disclosed in reference 1.

Reference 1 discloses that, by heating an Al—Si plated steel plate at 850° C. or more and forming a structure of a member with martensite through a hot-forming process and rapid cooling using a press, ultra-high strength with tensile strength of higher than 1600 MPa may be secured. Also, due to an alloying layer and a diffusion layer formed by diffusing Fe from a base material to a plating layer during heat treatment, corrosion-resistance and spot-weldability may be secured without a shot blasting process.

However, as an Al—Si plated layer needs to be formed, an additional plating process may be necessary, which may degrade economical efficiency and productivity.

In the case of a non-plated material, it may be impossible to secure spot-weldability due to an oxide layer created during heat treatment. Accordingly, a shot blasting process may be required to remove the oxide layer, and it may be difficult to secure corrosion-resistance.

Thus, it has been required to develop a cold-rolled steel plate for hot forming, which may secure excellent corrosion-resistance and spot-weldability without performing a plating process and a shot blasting process, a hot-formed member, and a method for manufacturing the same.

PRIOR ART

(Reference 1) U.S. Pat. No. 6,296,805

DISCLOSURE

Technical Problem

An aspect of the present disclosure is to provide a cold-rolled steel plate for hot forming, having excellent corrosion-resistance and spot-weldability without a plating process and a shot blasting process, a hot-formed member, and a method for manufacturing the same, which may be preferably applied to structural members, reinforcements, and the like, of vehicles in which crashworthiness is required.

Meanwhile, the purposes of the present disclosure are not limited to the features described above. The purposes of the present disclosure may be understood on the basis of the descriptions in the specification, and it may not be difficult

for a person having skilled in the art in the field in which the present disclosure is included to understand additional purposes of the present disclosure.

5 Technical Solution

An aspect of the present disclosure relates to a cold-rolled steel plate for hot forming, which is excellent in corrosion-resistance and spot-weldability, contains, by weight %, C: 0.1-0.4%, Si: 0.5-2.0%, Mn: 0.01-4.0%, Al: 0.001-0.4%, P: 0.001-0.05%, S: 0.0001-0.02%, Cr: 0.5% or higher and less than 3.0%, N: 0.001-0.02%, and a balance of Fe and inevitable impurities, satisfying formula (1) below, and includes an Si amorphous oxidation layer continuously or discontinuously formed to a thickness of 1 nm-100 nm on the surface thereof. Formula (1):  $1.4 \leq 0.4 \times Cr + Si \leq 3.2$  (wherein element symbols denote measurements of respective element contents by weight %).

10 Another aspect of the present disclosure relates to a method of manufacturing a cold-rolled steel plate for hot-forming, having excellent corrosion-resistance and spot-weldability, the method including, heating a slab to 1000-1300° C., the slab including C: 0.1 to 0.4%, Si: 0.5 to 2.0%, Mn: 0.01 to 4.0%, Al: 0.001 to 0.4%, P: 0.001 to 0.05%, S: 0.0001 to 0.02%, Cr: 0.5% or higher and less than 3.0%, N: 0.001 to 0.02%, and a balance of Fe and inevitable impurities by weight % and satisfying equation (1) below: equation (1):  $1.4 \leq 0.4 \times Cr + Si \leq 3.2$ , where each element symbol is a value of a content of each element measured by weight %; obtaining a hot-rolled steel plate by hot-rolling the heated slab at finishing rolling temperature of Ar3 to 1000° C.; coiling the hot-rolled steel plate within a temperature range of higher than Ms to 750° C. or less;

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 966

FIG. 2 is (a) a graph illustrating changes in thickness of an Si-based amorphous oxide layer of a cold-rolled steel plate in accordance with a value of equation (2), and (b) a graph illustrating changes in thickness of an Fe, Mn, and Cr oxide layer of a cold-rolled steel plate in accordance with a value of equation (3);

FIG. 3 is (a) a graph illustrating changes in thickness of an Si-based amorphous oxide layer of a hot-formed member in accordance with a value of equation (4), and (b) a graph illustrating changes in thickness of an Fe, Mn, and Cr oxide layer of a hot-formed member in accordance with a value of equation (5);

FIG. 4 is an image of a surface layer structure of embodiment A2 of a cold-rolled steel plate;

FIG. 5 is images of distributions of surface layer components of embodiment A2 of a cold-rolled steel plate;

FIG. 6 is an image of a surface layer structure of embodiment A2 of a hot-formed member; and

FIG. 7 is images of distributions of surface layer components of embodiment A2 of a hot-formed member.

#### BEST MODE FOR INVENTION

Hereinafter, embodiments of the present disclosure will be described with reference to the accompanied drawings. The present disclosure, however, may be modified to various other embodiments, and the scope of the present disclosure may not be limited to exemplary embodiments described below. These embodiments are provided to help those skilled in the art to understand the present disclosure.

In the case of a non-plated cold-rolled steel plate for hot forming, spot-weldability may not be secured due to an oxide layer formed during heat treatment, and a shot blasting process for removing the oxide layer may be required. Also, it may be difficult to secure corrosion-resistance. The purpose of the present disclosure is to address the issues above.

According to the present disclosure, by accurately controlling an alloy composition and manufacturing conditions, particularly by controlling the correlation among a content of Cr, a content of Si, and a dew point temperature, an Si-based amorphous oxide layer may be formed with a desired thickness such that, without a plating process and a shot blasting process, excellent corrosion-resistance and spot-weldability may be secured.

In the descriptions below, a cold-rolled steel plate for hot forming, having excellent corrosion-resistance and spot-weldability, will be described in accordance with an exemplary embodiment.

A cold-rolled steel plate for hot forming, having excellent corrosion-resistance and spot-weldability may include C: 0.1 to 0.4%, Si: 0.5 to 2.0%, Mn: 0.01 to 4.0%, Al: 0.001 to 0.4%, P: 0.001 to 0.05%, S: 0.0001 to 0.02%, Cr: 0.5% or higher and less than 3.0%, N: 0.001 to 0.02%, and a balance of Fe and inevitable impurities by weight %, and may satisfy equation (1) below. An Si-based amorphous oxide layer having a thickness of 1 nm to 100 nm may be continuously or discontinuously formed on a surface of the cold-rolled steel plate.

$$1.4 \leq 0.4 * Cr + Si \leq 3.2$$

Equation (1):

(where each element symbol is a value of a content of each element measured by weight %)

In the description below, an alloy composition of a cold-rolled steel plate for hot forming, having excellent corrosion-resistance and spot-weldability, will be described in greater detail in accordance with an exemplary embodiment. A unit of a content of each element may be weight %.

C: 0.1 to 0.4%

An appropriate content of C may be added as an essential element to improve strength of a heat treatment member.

When a content of C is less than 0.1%, it may be difficult to secure sufficient strength. Thus, a preferable content of C may be 0.1% or higher. When a content of C exceeds 0.4%, strength of a hot-rolled material may be excessively high when the hot-rolled material is cold-rolled, such that cold-rolling properties may be significantly deteriorated, and spot-weldability may also significantly degrade. Thus, a preferable content of C may be 0.4% or less. A more preferable upper limit may be 0.35%, and an even more preferable upper limit may be 0.3%.

Si: 0.5 to 2.0%

Si may be important in that Si is concentrated on a surface of the cold-rolled steel plate and forms an Si-based amorphous oxide layer when the cold-rolled steel plate is annealed on a continuous annealing line. Si may also prevent the formation of an Fe, Mn, and Cr oxide layer in a hot-forming process such that Si may secure spot-weldability of a member.

When a content of Si is less than 0.5%, the above-described effect may not be sufficient. Thus, a lower limit of a content of Si may be 0.5% preferably. A more preferable lower limit may be 0.8%. When a content of Si exceeds 2.0%, a thickness of an Si-based amorphous oxide layer may excessively increase such that spot-weldability may degrade.

Cr: 0.5% or Higher and Less than 3.0%

Cr may improve hardenability of a steel plate, and may help an Si-based amorphous oxide layer to be stably formed on a surface layer by appropriate reacting with Si.

When a content of Cr is less than 0.5%, the above-described effect may not be sufficient. When a content of Cr is 3.0% or higher, the effect may be saturated, and manufacturing costs may increase.

Cr and Si may need to satisfy the respective element contents described above, and may also need to satisfy equation (1):  $1.4 \leq 0.4 * Cr + Si \leq 3.2$ . As illustrated in FIG. 1, when a value of equation (1) is less than 1.4, it may be difficult to secure a uniform surface grade on a surface after a hot-forming process, and when a value of equation (1) exceeds 3.2, the effect may be saturated, and manufacturing costs may increase, and spot-weldability may degrade. A more preferable upper limit of a value of equation (1) may be 3.0, and an even more preferable upper limit may be 2.5.

Mn: 0.01 to 4.0%

Mn may be added to secure a solid solution strengthening effect and to reduce a critical cooling speed for securing martensite in relation to a hot-formed member.

When a content of Mn is less than 0.01%, the above-described effect may not be sufficient. When a content of Mn exceeds 4.0%, strength of a steel plate before a hot-forming process may excessively increase such that it may be difficult to perform a blanking process. Further, due to excessive addition of ferro-alloy, costs of raw materials may rise, and spot-weldability may degrade. A more preferable upper limit may be 3.0%, and an even more preferable upper limit may be 2.0%.

Al: 0.001 to 0.4%

Al may perform deoxidization in steelmaking along with Si, and may increase cleanliness of steel accordingly.

When a content of Al is less than 0.001%, the above-described effect may not be sufficient, and when a content of Al exceeds 0.4%, an Ac3 temperature may excessively rise such that a heating temperature may need to be increased. A

more preferable upper limit may be 0.2%, and an even more preferable upper limit may be 0.1%.

P: 0.001 to 0.05%

P may be impurities. To control a content of P to be less than 0.001%, relatively high manufacturing costs may be required. When a content of P exceeds 0.05%, weldability of a hot-formed member may significantly degrade. A more preferable upper limit may be 0.03%.

S: 0.0001 to 0.02%

S may be impurities. To control a content of S to be less than 0.0001%, relatively high manufacturing costs may be required. When a content of S exceeds 0.02%, ductility of a member, impact toughness, and weldability may degrade. A more preferable upper limit may be 0.01%.

N: 0.001 to 0.02%

N may be impurities. To control a content of N to be less than 0.001%, relatively high manufacturing costs may be required. When a content of N exceeds 0.02%, a slab may become vulnerable to cracks when the slab is continuously casted, and impact toughness may be deteriorated. A more preferable upper limit may be 0.01%.

A remaining element of the exemplary embodiment may be iron (Fe). In a general manufacturing process, as unintended impurities from raw materials or surrounding environment may inevitably be mixed, impurities may not be excluded. A person skilled in the art, familiar with a general manufacturing process, may be aware of the impurities, and thus, the impurities will not be described in greater detail.

In addition to the above-described elements, one or more elements selected from between a) and b) may further be included.

a) One or More Elements Selected from Among Ti, Nb, Zr, and V: 0.001 to 0.4%

Ti, Nb, Zr, and V may form fine precipitations, which may be effective to improve strength of a heat treatment member, and may also be effective to stabilize residual austenite and to improve impact toughness due to grain refinement. When a content (a sum of contents of Ti, Nb, Zr, and V when two or more elements are added) of Ti, Nb, Zr, and V is 0.001% or lower, the above-described effect may not be sufficient. When a content of Ti, Nb, Zr, and V exceeds 0.4%, the effect may be saturated, and due to excessive addition of ferro-alloy, costs of raw materials may also increase.

b) B: 0.0001 to 0.01%

With even a small content of B, B may improve hardenability. Also, B may be segregated into grain boundaries of prior austenite such that B may prevent brittleness of the hot-formed member by grain boundary segregation of P and/or S.

When a content B is less than 0.0001%, the above-described effect may not be sufficient. When a content of B exceeds 0.01%, the effect may be saturated, and hot brittleness may occur when a hot-rolling process is performed. A more preferable upper limit may be 0.005%.

Also, one or more elements selected from among c) to e) may further be included.

c) One or More Elements Selected from Between Mo and W: 0.001 to 1.0%

Mo and W may be added to improve hardenability, and to improve strength through a precipitation reinforcement effect and to obtain grain refinement. When a content (a sum of contents of Mo and W when both of Mo and W are added) of Mo and W is less than 0.001%, the above-described effect may not be sufficient. When a content of Mo and W exceeds 1.0%, the effect may be saturated, and costs may rise.

d) A Sum of Contents of Cu and Ni: 0.005 to 2.0%

Cu may be added as an element which improves strength by forming fine precipitations. When Cu is added alone, it may cause hot brittleness, and thus, Ni may be added if necessary.

When a sum of contents of Cu and Ni is less than 0.005%, the above-described effect may not be sufficient. When a sum of the contents exceeds 2.0%, costs may rise excessively.

10 e) One or More Elements Selected from Between Sb and Sn: 0.001 to 1.0%

Sb and Sn may be effective to prevent the formation of oxide which may be formed on grain boundaries on a surface layer of a hot-rolled material of steel to which Si is added, such that Sb and Sn may prevent dent defects caused by separation of grain boundaries on a surface layer when a cold rolled material is annealed. To obtain such an effect, a preferable content of Sb and Sn may be 0.001% or higher.

When a content (a sum of contents of Sb and Sn when both of Sb and Sn are added) of Sb and Sn exceeds 1.0%, costs may rise excessively. Further, Sb and Sn may be solidified to grain boundaries of a slab, which may cause cracks on coil edges when a hot-rolling process is performed.

25 20 25 The cold-rolled steel plate for hot-forming, having excellent corrosion-resistance and spot-weldability, in the exemplary embodiment may satisfy the above-described alloy composition, and an Si-based amorphous oxide layer having a thickness of 1 to 100 nm may be formed continuously or discontinuously on a surface of the steel plate.

30 The Si-based amorphous oxide layer may be oxide created when Si is combined with oxygen, and may refer to a layer formed of oxide having an amorphous structure, which may be created when Si added to steel is concentrated onto a surface layer and is combined with oxygen in a furnace during an annealing process. The Si-based amorphous oxide layer may be strong against corrosion, and may be effective to improve corrosion-resistance and to prevent the formation of an Fe, Mn, and Cr oxide layer.

40 35 40 When a thickness of the Si-based amorphous oxide layer is less than 1 nm, it may be difficult to form a sufficient Si-based amorphous oxide layer after a hot-forming process. Accordingly, the effect of improvement in corrosion-resistance may be insignificant, and the formation of an Fe, Mn, and Cr oxide layer may be facilitated such that it may be difficult to secure sufficient corrosion-resistance and good spot-weldability.

45 50 45 When a thickness of the Si-based amorphous oxide layer exceeds 100 nm, sufficient corrosion-resistance may be secured after a hot-forming process, but it may be difficult to secure spot-weldability. Thus, a preferable upper limit of a thickness of the Si-based amorphous oxide layer may be 100 nm, a more preferable upper limit may be 70 nm, and an even more preferable upper limit may be 50 nm.

55 55 In this case, the Fe, Mn, and Cr oxide layer may be formed to a thickness of 2.5  $\mu\text{m}$  or less on the Si-based amorphous oxide layer.

When a thickness of the Fe, Mn, and Cr oxide layer exceeds 2.5  $\mu\text{m}$ , a shot blasting process may be required to 60 remove the Fe, Mn, and Cr oxide layer so as to secure spot-weldability, and it may be difficult to secure corrosion-resistance.

65 A microstructure of the cold-rolled steel plate in the exemplary embodiment may include ferrite and cementite. In particular, it may not be necessary to limit an area fraction of the microstructure. For example, an area fraction of ferrite and cementite may be 50 area % or more.

When a blank is made to manufacture a hot-formed member, if strength of the cold-rolled steel plate is too high, mold abrasion may easily occur. However, without considering the mold abrasion, bainite, martensite, and the like, may be included.

In the description below, a method of manufacturing a cold-rolled steel plate for hot-forming will be described in detail in accordance with an exemplary embodiment.

A method of manufacturing a cold-rolled steel plate for hot-forming according to an exemplary embodiment may include heating a slab satisfying the above-described alloy composition to 1000 to 1300° C.; obtaining a hot-rolled steel plate by hot-rolling the heated slab at finishing rolling temperature of Ar3 to 1000° C.; coiling the hot-rolled steel plate at a temperature range of higher than Ms to 750° C. or less; obtaining a cold-rolled steel plate by cold-rolling the coiled hot-rolled steel plate; and continuously annealing the cold-rolled steel plate to satisfy equation (2) and equation (3) below:

$$1.4 \leq 0.4 * Cr + Si \leq 3.2 \quad \text{Equation (1):}$$

$$1 \leq \exp [0.07 * DP(I) + (0.6 * Cr + 3 * Si)] \leq 100 \quad \text{Equation (2):}$$

$$50 * \exp [0.05 * DP(I) - (1.2 * Cr + 6 * Si)] \leq 2.5 \quad \text{Equation (3):}$$

(in equation (1) to equation (3), each element symbol is a value of a content of each element measured by weight %, and in equation (2) and equation (3), DP(I) is a dew point temperature when the continuous annealing is performed).

#### Heating Slab

A slab satisfying the above-described alloy composition may be heated to 1000 to 1300° C.

When the heating temperature is less than 1000° C., it may be difficult to homogenize a structure of the slab. When the heating temperature exceeds 1300° C., oxide may be excessively formed, and manufacturing costs may rise.

#### Hot-Rolling

A hot-rolled steel plate may be obtained by hot-rolling the heated slab at finishing rolling temperature of Ar3 to 1000° C.

When the finishing rolling temperature is less than an Ar3 temperature, the rolling may be performed at two phase regions such that duplex grain structures may be created on a surface layer, and it may be difficult to control a shape of the hot-rolled steel plate. When the finishing rolling temperature exceeds 1000° C., grains of the hot-rolled steel plate may easily be coarsened.

#### Coiling

The hot-rolled steel plate may be coiled at a temperature range of higher than Ms to 750° C. or less.

When the coiling temperature is Ms (a martensite transformation initiating temperature) or lower, strength of the hot-rolled steel plate may be excessively high such that cold-rolling properties may degrade. When the coiling temperature exceeds 750° C., a thickness of an oxide layer may increase, and grain boundary oxidation may occur on a surface layer such that pickling properties may degrade, and separation of grain boundaries on a surface layer may occur during an annealing process in a continuous annealing furnace.

#### Cold-Rolling

A cold-rolled steel plate may be obtained by cold-rolling the coiled hot-rolled steel plate. This process may be performed to more accurately control a thickness of the steel plate, and a pickling process may be performed before the cold-rolling.

It may not be necessary to limit a reduction ratio of the cold-rolling to a particular value, but to secure a certain target thickness, a reduction ratio may be 30 to 80%.

#### Continuous Annealing

The cold-rolled steel plate may be continuously annealed to satisfy equation (2) and equation (3) below. In equation (2) and equation (3), each element symbol is a value of a content of each element measured by weight %, and DP(I) is a dew point temperature when the continuous annealing is performed.

$$1 \leq \exp [0.07 * DP(I) + (0.6 * Cr + 3 * Si)] \leq 100 \quad \text{Equation (2):}$$

Equation (2) may be to control a thickness of the Si-based amorphous oxide layer of the cold-rolled steel plate in consideration of correlation among a content of Si, a content of Cr, and a dew point (DP(I)) of when the continuous annealing is performed. As indicated in FIG. 2(a), graphs illustrating changes in thickness of the Si-based amorphous oxide layer of the cold-rolled steel plate in accordance with a value of equation (2), a thickness of the Si-based amorphous oxide layer may be controlled in accordance with a value of equation (2).

When a value of equation (2) is less than 1, a sufficient thickness of the Si-based amorphous oxide layer may not be secured on a surface such that it may be difficult to prevent the formation of an Fe, Mn, and Cr oxide layer, and without an additional plating process or a shot blasting process, excellent spot-weldability and corrosion-resistance may not be secured.

When a value of equation (2) exceeds 100, a thickness of the Si-based amorphous oxide layer may excessively increase such that it may be difficult to secure sufficient spot-weldability.

$$50 * \exp [0.05 * DP(I) - (1.2 * Cr + 6 * Si)] \leq 2.5 \quad \text{Equation (3):}$$

Equation (3) is to control a thickness of the Fe, Mn, and Cr oxide layer of the cold-rolled steel plate in consideration of correlation among a content of Si, a content of Cr, and a dew point (DP(I)) of when the continuous annealing is performed. As indicated in FIG. 2(b), graphs illustrating changes in thickness of the Si-based amorphous oxide layer of the cold-rolled steel plate in accordance with a value of equation (3), a thickness of the Fe, Mn, and Cr oxide layer may be controlled in accordance with a value of equation (3).

When a value of equation (3) exceeds 2.5, a thickness of the Fe, Mn, and Cr oxide layer may increase such that an exterior of a surface of the steel plate may be deteriorated, and spot-weldability may also be deteriorated after a hot-forming process.

The continuous annealing may be performed within a temperature range of 700 to 900° C. When an annealing temperature is less than 700° C., it may be difficult to restore and recrystallize a rolled structure created by the cold-rolling. When an annealing temperature exceeds 900° C., an annealing facility may be deteriorated, and excessive oxide may be formed on a surface layer of the steel plate, which may significantly degrade spot-weldability after the hot-forming.

An annealing time may be 1 to 1000 seconds. In the exemplary embodiment, as an annealing process is continuously performed, it may be difficult to accurately control the annealing time, and thus, a dew point may be controlled. When the annealing time is less than 1 second, it may be difficult to obtain an annealing effect, and when the annealing time exceeds 1000 seconds, productivity may degrade.

In the description below, a method of manufacturing a hot-formed member having excellent corrosion-resistance and spot-weldability will be described in detail in accordance with an exemplary embodiment.

A method of manufacturing a hot-formed member having excellent corrosion-resistance and spot-weldability in the exemplary embodiment may include performing heat treatment in which a cold-rolled steel plate manufactured by the method of manufacturing the cold-rolled steel plate described in the aforementioned exemplary embodiment is heated to a temperature range of Ac3 to Ac3+150° C. at a temperature rising speed of 1 to 1000° C./sec while satisfying equation (4) and equation (5) below, and the heated cold-rolled steel plate is maintained for 1 to 1000 seconds; and hot-forming the heated cold-rolled steel plate and cooling the steel plate at a cooling speed of 10 to 1000° C./sec.

#### Heat Treatment

In the heat treatment, the cold-rolled steel plate manufactured by the method of manufacturing the cold-rolled steel plate in the aforementioned exemplary embodiment may be heated to a temperature range of Ac3 to Ac3+150° C. at a temperature rising speed of 1 to 1000° C./sec while satisfying equation (4) and equation (5) below, and the heated cold-rolled steel plate may be maintained for 1 to 1000 seconds.

When the temperature rising speed is less than 1° C./sec, it may be difficult to secure sufficient productivity, and oxidation may be accelerated excessively on a surface of the member such that it may be difficult to secure sufficient spot-weldability. When the temperature rising speed exceeds 1000° C./sec, an expensive facility may be required.

When the heating temperature is less than Ac3, or the maintaining time is less than 1 second, ferrite which has not been completely transformed to austenite may remain, and ferrite may be formed again while a blank is transferred to a mold from a heating furnace such that it may be difficult to secure a certain strength. When the heating temperature exceeds Ac3+150° C., or the maintaining time exceeds 1000 seconds, oxide may be excessively formed on a surface of the member such that it may be difficult to secure spot-weldability.

In equation (4) and equation (5), each element symbol is a value of a content of each element measured by weight %, and DP(II) is a dew point temperature of the heat treatment.

$$2 \leq \text{equation (2)} \cdot \exp [0.07 \cdot \text{DP(II)} + (0.6 \cdot \text{Cr} + 1.5 \cdot \text{Si})] \leq 2000 \quad \text{Equation (4):}$$

Equation (4) may be to control a thickness of the Si-based amorphous oxide layer of the hot-formed member in consideration of correlation among a content of Si, a content of Cr, a dew point (DP(I)) of when the continuous annealing is performed, and a dew point (DP(II)) of when the heat treatment is performed. As indicated in FIG. 3(a), graphs illustrating changes in thickness of the Si-based amorphous oxide layer of the hot-formed member in accordance with a value of equation (4), a thickness of the Si-based amorphous oxide layer of the hot-formed member may be controlled in accordance with a value of equation (4).

When a value of equation (4) is less than 2, it may be difficult to secure a sufficient thickness of the Si-based amorphous oxide layer on a surface such that sufficient corrosion-resistance may not be secured. Thus, a preferable lower limit of a value of equation (4) may be 2, a more preferable value may be 3, and an even more preferable value may be 4.

When a value of equation (4) exceeds 2000, a thickness of the Si-based amorphous oxide layer may excessively increase such that it may be difficult to sufficient spot-weldability.

5  $2 \leq \text{equation (3)} + 50 \cdot \exp [0.05 \cdot \text{DP(II)} - (0.4 \cdot \text{Cr} + 2 \cdot \text{Si})] \leq 3 \quad \text{Equation (5):}$

Equation (5) may be to control a thickness of the Fe, Mn, and Cr oxide layer of the hot-formed member in consideration of correlation among a content of Si, a content of Cr, and a dew point (DP(I)) of when the continuous annealing is performed, and a dew point (DP(II)) of when the heat treatment is performed. As indicated in FIG. 3(b), graphs illustrating changes in thickness of the Fe, Mn, and Cr oxide layer of the hot-formed member in accordance with a value of equation (5), a thickness of the Fe, Mn, and Cr oxide layer of the hot-formed member may be controlled in accordance with a value of equation (5).

When a value of equation (5) exceeds 3, a thickness of the Fe, Mn, and Cr oxide layer may increase such that an exterior of a surface of the steel plate may be deteriorated, and spot-weldability may degrade.

#### Hot-Forming and Cooling

After hot-forming the heated cold-rolled steel plate, the steel plate may be cooled at a cooling speed of 10 to 1000° C./sec.

When the cooling speed is less than 10° C./sec, unwanted ferrite may be formed such that it may be difficult to secure 1000 MPa or higher tensile strength, whereas, to control the cooling speed to exceed 1000° C./sec, an extensive and special cooling facility may be required.

A cooling stop temperature of the cooling may be Mf (a martensite transformation terminating temperature) or less.

35 When the cooling stops at a temperature higher than Mf, and the cooling is performed again to cool down the steel plate to room temperature, it may be difficult to secure shape fixability of the hot-formed member.

However, to secure improved elongation and impact 40 toughness of the hot-formed member, the cooling may stop between Mf (a martensite transformation terminating temperature) and Ms (a martensite transformation initiating temperature), and the steel plate may be heated again at temperature of Ac1 or lower such that martensite may be tempered and residual austenite may be stabilized.

In the description below, a hot-formed member having excellent corrosion-resistance and spot-weldability will be described in detail in accordance with an exemplary embodiment.

50 The hot-formed member having excellent corrosion-resistance and spot-weldability in the exemplary embodiment may satisfy the above-described alloy composition, and an Si-based amorphous oxide layer having a thickness of 2 nm to 2000 nm may be continuously or discontinuously formed on a surface of the hot-formed member.

When a thickness of the Si-based amorphous oxide layer is less than 2 nm, it may be difficult to secure sufficient corrosion-resistance. Thus, a lower limit of the thickness may be 2 nm preferably, a more preferable lower limit may be 3 nm, and an even more preferable lower limit may be 3.5 nm.

60 When the thickness exceeds 2000 nm, sufficient corrosion-resistance may be secured, but it may be difficult to secure sufficient spot-weldability. Thus, an upper limit of the thickness may be 2000 nm preferably, a more preferable upper limit may be 1000 nm, and an even more preferable upper limit may be 500 nm.

## 11

An Fe, Mn, and Cr oxide layer may be formed to a thickness of 3  $\mu\text{m}$  or less on the Si-based amorphous oxide layer.

When a thickness of the Fe, Mn, and Cr oxide layer exceeds 3  $\mu\text{m}$ , an exterior of a surface of the steel plate may be deteriorated, and a shot blasting process for removing the Fe, Mn, and Cr oxide layer may be required to secure spot-weldability, and it may be difficult to secure corrosion-resistance.

To secure high strength, the hot-formed member may include martensite or bainite as a main phase. The main phase refers to a phase having the largest area fraction among numerous phases forming a microstructure. The area fraction may not be limited to a particular value. For example, the area fraction may be 50 area % or higher.

The hot-formed member may have 1000 MPa or higher tensile strength. By securing 1000 MPa or higher tensile strength, the hot-formed member may be applied to structural members or reinforcements of vehicles in which crash-worthiness is required.

The hot-formed member may have a spot welding current range of 1.0 kA or higher. When the spot welding current range is 1.0 kA, spot-weldability may be deteriorated, and generally, most of customer companies require a spot welding current range of 1.0 kA or higher.

## MODE FOR INVENTION

In the description below, embodiments of the present disclosure will be described in greater detail. It should be noted that the exemplary embodiments are provided to describe the present disclosure in greater detail, and to not limit the scope of rights of the present disclosure. The scope of rights of the present disclosure may be determined on the basis of the subject matters recited in the claims and the matters reasonably inferred from the subject matters.

## Embodiment 1

In the embodiment, a slab having element composition indicated in table 1 and having a thickness of 40 mm was melted in vacuum, heated at 1200° C. for 1 hour in a heating furnace, hot-rolled at a finishing rolling temperature of 900° C., and a hot-rolled steel plate having a final thickness of 3 mm was manufactured. The hot-rolled steel plate was coiled at 600° C. Thereafter, the hot-rolled steel plate was pickled, and the hot-rolled steel plate was cold-rolled at a cold reduction ratio of 50%.

Using the cold-rolled steel plate manufactured as above, a continuous annealing process was performed while varying a dew point condition (DP(I)) at an annealing temperature of 780° C. as in table 2. After the continuous annealing process, a thickness of an Si-based amorphous oxide layer and a thickness of an Fe, Mn, and Cr oxide layer formed on a surface of the cold-rolled steel plate were measured and listed in table 2 below. Also, values of equation (1) to equation (3) were calculated and listed in table 3.

$$1.4 \leq 0.4 * \text{Cr} + \text{Si} \leq 3.2 \quad \text{Equation (1):}$$

$$1 \leq \exp [0.07 * \text{DP(I)} + (0.6 * \text{Cr} + 3 * \text{Si})] \leq 100 \quad \text{Equation (2):}$$

$$50 * \exp [0.05 * \text{DP(I)} - (1.2 * \text{Cr} + 6 * \text{Si})] \leq 2.5 \quad \text{Equation (3):}$$

(In equation (1) to equation (3), each element symbol is a value of a content of each element measured by weight %, and in equation (2) and equation (3), DP(I) is a dew point temperature when the continuous annealing is performed).

## 12

A thickness of the Si-based amorphous oxide layer and a thickness of the Fe, Mn, and Cr oxide layer were indicated by result values obtained by averaging thicknesses of three regions measured using a transmission electron microscope (TEM) and an EPMA device. FIGS. 4 and 5 are images showing a representative surface layer structure and a composition distribution of embodiment A2. Embodiments A1 to A4 satisfy equation (2) and equation (3), whereas embodiments A5 and A6 and B1 to B5 do not satisfy equation (2) or equation (3).

Using the cold-rolled steel plate manufactured as above, a hot-forming process was performed, and as heat treatment conditions, a temperature of the heat treatment was controlled to be the dew point temperature (DP(II)) indicated in table 3 below, and after the steel plate was charged into a heating furnace which was heated to be 900° C. in advance, the steel plate was maintained for 6 minutes. Thereafter, the steel plate was air-cooled for 12 seconds, hot-formed in a mold, and rapidly cooled to room temperature at a cooling speed of 10° C./sec or higher, thereby obtaining a hot-formed member. Tensile strength, a surface grade, a thickness of the Si-based amorphous oxide layer, a thickness of the Fe, Mn, and Cr oxide layer, corrosion-resistance, and spot-weldability of the hot-formed member were measured or assessed, and the results are listed in table 3 below. Also, values of equation (4) and equation (5) were calculated and listed in table 3 below.

$$\begin{aligned} 2 \leq \text{equation} & (2) * \exp [0.6 * \text{Cr} + 1.5 * \text{Si}] \leq 2000 \\ & [0.07 * \text{DP(II)} + \text{Equation (4):} \end{aligned}$$

$$\text{equation (3)} + 50 * \exp [0.05 * \text{DP(II)} - (0.4 * \text{Cr} + 2 * \text{Si})] \leq 3 \quad \text{Equation (5):}$$

(in equation (4) and equation (5), each element symbol is a value of a content of each element measured by weight %, and DP(II) is a dew point temperature (° C.) of the heat treatment).

The tensile strength was measured from an ASTM E8 tensile sample obtained from the hot-formed member, and a thickness of the Si-based amorphous oxide layer and a thickness of the Fe, Mn, and Cr oxide layer were indicated by result values obtained by averaging thicknesses of three regions measured using a transmission electron microscope (TEM) and an EPMA device. A representative surface layer structure and a composition distribution of embodiment A2-1 after hot-forming were indicated in FIGS. 6 and 7.

A surface grade was assessed by observing a surface onto which a shot blasting process was not performed by the naked eye. In other words, an area rate of the case in which a color of a surface looked dark grey as the surface of the member is formed of a thick oxide layer, and an area rate of the case in which a color of a surface appeared yellow or gold as the surface was formed of a thin oxide layer were calculated and assessed as below.

Grade 5: an area rate of a grey surface exceeds 90%

Grade 4: an area rate of a grey surface exceeds 70% and is 90% or less

Grade 3: an area rate of a grey surface exceeds 30% and is 70% or less

# US 11,441,205 B2

## 13

Grade 2: an area rate of a grey surface exceeds 10% and is 30% or less

Grade 1: an area rate of a grey surface is 10% or less

Corrosion-resistance was assessed by averaging values of corroded depths at three regions with 2 mm of intervals after performing a cyclic corrosion test (CCT) to the hot-formed member sixty three times using salt spray. In the embodiment in which the corroded depth exceeded 1 mm, the

## 14

embodiment was determined as defect (X), and when the corroded depth was 1 mm or less, the embodiment was determined as good (O).

Spot-weldability was assessed by calculating a spot welding current range using an ISO 18278-2 method. When the current range was 1.0 kA or higher, the embodiment was determined as good, and the current range was less than 1.0 kA, the embodiment was determined as a defect.

TABLE 1

| Chemical Composition (weight %) |      |      |      |       |       |      |      |      |        |       |        |              |                   |
|---------------------------------|------|------|------|-------|-------|------|------|------|--------|-------|--------|--------------|-------------------|
| Steel Type                      | C    | Si   | Mn   | P     | S     | Al   | Cr   | Ti   | B      | N     | Others | Equation (1) | Note              |
| A                               | 0.20 | 1.18 | 0.21 | 0.010 | 0.002 | 0.03 | 2.00 | 0.03 | 0.0025 | 0.004 | —      | 1.98         | Embodiment Steel  |
| B                               | 0.21 | 0.28 | 1.19 | 0.014 | 0.005 | 0.03 | 0.24 | 0.03 | 0.0024 | 0.004 | —      | 0.37         | Comparative Steel |
| C                               | 0.22 | 0.58 | 1.27 | 0.015 | 0.005 | 0.05 | 0.62 | 0.04 | 0.0019 | 0.003 | —      | 0.83         | Comparative Steel |

TABLE 2

| Cold-Rolled Steel Plate |                |               |                             |                         |              |              |                     |
|-------------------------|----------------|---------------|-----------------------------|-------------------------|--------------|--------------|---------------------|
| Steel type              | Classification | DP (I) (° C.) | Thickness of Amorphous (nm) | Thickness of Oxide (μm) | Equation (2) | Equation (3) | Note                |
| A                       | A1             | -50           | 2.7                         | 0.0003                  | 3.5          | 0.0003       | Embodiment          |
|                         | A2             | -30           | 16.5                        | 0.004                   | 14.0         | 0.001        | Embodiment          |
|                         | A3             | -20           | 25.7                        | 0.005                   | 28.2         | 0.001        | Embodiment          |
|                         | A4             | -10           | 65.7                        | 0.005                   | 56.8         | 0.002        | Embodiment          |
|                         | A5             | 0             | 120.1                       | 0.006                   | 114.4        | 0.004        | Comparative Example |
|                         | A6             | 10            | 198.7                       | 0.008                   | 230.4        | 0.006        | Comparative Example |
| B                       | B1             | -40           | 0.2                         | 0.7                     | 0.2          | 0.9          | Comparative Example |
|                         | B2             | -30           | 0.4                         | 1.3                     | 0.3          | 1.6          | Comparative Example |
|                         | B3             | -20           | 0.5                         | 2.4                     | 0.7          | 2.6          | Comparative Example |
|                         | B4             | -10           | 1.5                         | 3.8                     | 1.3          | 4.2          | Comparative Example |
|                         | B5             | 0             | 1.0                         | 9.2                     | 2.7          | 7.0          | Comparative Example |
| C                       | C1             | 30            | 58.0                        | 2.8                     | 67.5         | 3.3          | Comparative Example |

DP (I): a dew point temperature (° C.) of when a continuous annealing is performed

Amorphous: an Si-based amorphous oxide layer

Oxide: an Fe, Mn, and Cr oxide layer

TABLE 3

| Hot-Formed Member       |                |             |                        |               |                             |                         |              |              |                      |                                |                     |
|-------------------------|----------------|-------------|------------------------|---------------|-----------------------------|-------------------------|--------------|--------------|----------------------|--------------------------------|---------------------|
| Cold-Rolled Steel Plate | Classification | DP (II) (□) | Tensile Strength (MPa) | Surface Grade | Thickness of Amorphous (nm) | Thickness of Oxide (μm) | Equation (4) | Equation (5) | Corrosion-resistance | Range of Spot-Weldability (kA) | Note                |
| A1                      | A1-1           | -40         | 1513                   | 1.9           | 3.8                         | 0.32                    | 4.1          | 0.29         | O                    | 2.6                            | Embodiment          |
|                         | A1-2           | -60         | 1513                   | 1.0           | 1.8                         | 0.17                    | 1.0          | 0.11         | X                    | 2.8                            | Comparative Example |
| A1-3                    |                | 20          | 1513                   | 3.0           | 251.0                       | 5.8                     | 273.1        | 5.8          | O                    | 0                              | Comparative Example |
| A2                      | A2-1           | -30         | 1504                   | 1.8           | 27.5                        | 0.64                    | 33.45        | 0.47         | O                    | 1.8                            | Embodiment          |
| A3                      | A3-1           | -20         | 1527                   | 1.8           | 105.6                       | 0.78                    | 135.64       | 0.78         | O                    | 1.4                            | Embodiment          |
| A4                      | A4-1           | -10         | 1498                   | 1.8           | 504.8                       | 1.13                    | 550.04       | 1.29         | O                    | 1.2                            | Embodiment          |

TABLE 3-continued

| Hot-Formed Member       |                |             |                        |               |                             |                         |              |              |                      |                                |                     |
|-------------------------|----------------|-------------|------------------------|---------------|-----------------------------|-------------------------|--------------|--------------|----------------------|--------------------------------|---------------------|
| Cold-Rolled Steel Plate | Classification | DP (II) (□) | Tensile Strength (MPa) | Surface Grade | Thickness of Amorphous (nm) | Thickness of Oxide (μm) | Equation (4) | Equation (5) | Corrosion-resistance | Range of Spot-Weldability (kA) | Note                |
| A5                      | A5-1           | 0           | 1517                   | 1.3           | 2276.8                      | 1.84                    | 2230.54      | 2.12         | ○                    | 0.4                            | Comparative Example |
| A6                      | A6-1           | 10          | 1508                   | 1.3           | 8724.1                      | 3.87                    | 9045.29      | 3.50         | ○                    | 0.2                            | Comparative Example |
| B1                      | B1-1           | 0           | 1534                   | 5.0           | 0.3                         | 23.5                    | 0.28         | 27.1         | X                    | 0.2                            | Comparative Example |
| B2                      | B2-1           | 0           | 1528                   | 5.0           | 0.5                         | 25.1                    | 0.57         | 27.8         | X                    | 0                              | Comparative Example |
| B3                      | B3-1           | 0           | 1543                   | 5.0           | 1.3                         | 26.2                    | 1.14         | 28.8         | X                    | 0                              | Comparative Example |
| B4                      | B4-1           | 0           | 1527                   | 5.0           | 2.5                         | 27.1                    | 2.29         | 30.5         | ○                    | 0                              | Comparative Example |
| B5                      | B5-1           | 0           | 1515                   | 5.0           | 4.3                         | 31.5                    | 4.62         | 33.3         | ○                    | 0                              | Comparative Example |
| C1                      | C1-1           | 0           | 1575                   | 4.0           | 250.0                       | 14.5                    | 233.7        | 15.5         | ○                    | 0                              | Comparative Example |

DP (I): a dew point temperature (°C.) of heat treatment

Amorphous: an Si-based amorphous oxide layer

Oxide: an Fe, Mn, and Cr oxide layer

25 A grade of embodiment steel A satisfying a value of equation (1) was less than grade 4 under overall heat treatment conditions in the hot-forming process.

A surface grade of comparative steel B which does not satisfy values of Si, Cr, and equation (1) was grade 5 under heat treatment conditions in the hot-forming process, which indicates that surface properties were deteriorated. A surface grade of embodiment steel C, of which a range of a content of each element satisfies the range of the exemplary embodiment but which does not satisfy a value of equation (1), was grade 4, which indicates that surface properties were deteriorated.

Also, using embodiments A1 to A4, a hot-formed member which may secure both corrosion-resistance and spot-weldability was made.

Comparative examples A5 and A6 which satisfy the alloy composition of the exemplary embodiment but which do not satisfy the conditions of a cold-rolled steel plate of the exemplary embodiment were able to secure corrosion-resistance, but were not able to secure spot-weldability.

Comparative example A1-2 satisfied the conditions of a cold-rolled steel plate of the exemplary embodiment, but a value of equation (4) was less than 2, and accordingly, corrosion-resistance of the hot-formed member was deteriorated. Comparative example A1-3 satisfied the conditions of a cold-rolled steel plate of the exemplary embodiment, but

30 a value of equation (5) exceeded 3, and accordingly, spot-weldability of the hot-formed member was deteriorated.

## Embodiment 2

To further check that 1000 MPa or higher tensile strength, and excellent corrosion-resistance and spot-weldability may be secured within the range of the exemplary embodiment, and addition experiments were conducted.

35 Using a slab having composition as in table 4 and having a thickness of 40 mm, a cold-rolled steel plate and a hot-formed member were manufactured under conditions of a dew point temperature of when a continuous annealing process was performed in table 5 below, a dew point temperature of heat treatment in table 6 below, and other manufacturing conditions as in embodiment 1 above.

40 A thickness of an Si-based amorphous oxide layer and a thickness of an Fe, Mn, and Cr oxide layer formed on a surface of the cold-rolled steel plate were measured and listed in table 5 below.

45 Tensile strength, a surface grade, a thickness of the Si-based amorphous oxide layer, a thickness of the Fe, Mn, and Cr oxide layer, corrosion-resistance, and spot-weldability of the hot-formed member were measured or assessed, and listed in table 6 below.

50 The measuring method and the assessment method were the same as in embodiment 1 above.

TABLE 4

| Steel | Chemical Composition (Weight %) |      |      |        |        |       |      |       |        |        |                      |        |                  |
|-------|---------------------------------|------|------|--------|--------|-------|------|-------|--------|--------|----------------------|--------|------------------|
|       | Type                            | C    | Si   | Mn     | P      | s     | Al   | Cr    | Ti     | B      | N                    | Others | Equation (1)     |
| D     | 0.19                            | 1.24 | 3.0  | 0.0070 | 0.0025 | 0.035 | 1.21 | —     | —      | 0.0040 | —                    | 1.72   | Embodiment Steel |
| E     | 0.21                            | 1.21 | 0.06 | 0.0071 | 0.0025 | 0.028 | 2.09 | 0.030 | 0.0025 | 0.0040 | Nb: 0.03             | 2.05   | Embodiment Steel |
| F     | 0.21                            | 1.24 | 0.22 | 0.0110 | 0.0025 | 0.034 | 2.03 | 0.033 | 0.0027 | 0.0041 | Ni: 0.15<br>Cu: 0.51 | 2.05   | Embodiment Steel |
| G     | 0.21                            | 1.18 | 0.80 | 0.0071 | 0.0025 | 0.024 | 0.79 | 0.030 | 0.0025 | 0.0040 | Mo: 0.15             | 1.50   | Embodiment Steel |
| H     | 0.21                            | 1.64 | 0.46 | 0.0074 | 0.0024 | 0.035 | 1.15 | 0.030 | 0.0025 | 0.0040 | V: 0.05              | 2.10   | Embodiment Steel |

TABLE 4-continued

| Steel |      |      |      |        |        |       |      |       |        |        |          |              | Chemical Composition (Weight %) |  |
|-------|------|------|------|--------|--------|-------|------|-------|--------|--------|----------|--------------|---------------------------------|--|
| Type  | C    | Si   | Mn   | P      | s      | Al    | Cr   | Ti    | B      | N      | Others   | Equation (1) | Note                            |  |
| I     | 0.21 | 1.17 | 0.81 | 0.0073 | 0.0025 | 0.027 | 0.80 | 0.030 | 0.0025 | 0.0040 | Sb: 0.03 | 1.49         | Embodiment Steel                |  |
| J     | 0.21 | 1.13 | 0.68 | 0.0086 | 0.0028 | 0.025 | 0.76 | 0.030 | 0.0027 | 0.0038 | Sn: 0.03 | 1.43         | Embodiment Steel                |  |
| K     | 0.21 | 1.15 | 0.92 | 0.0113 | 0.0017 | 0.054 | 0.85 | 0.030 | 0.0026 | 0.0024 | W: 0.03  | 1.49         | Embodiment Steel                |  |

TABLE 5

| Cold-Rolled Steel Plate |    |               |                                   |                               |                 |                 |            |
|-------------------------|----|---------------|-----------------------------------|-------------------------------|-----------------|-----------------|------------|
| I                       | fi | DP (I)<br>(□) | Thickness of<br>Amorphous<br>(nm) | Thickness<br>of Oxide<br>(μm) | Equation<br>(2) | Equation<br>(3) | Note       |
| D                       | D1 | -30           | 13.4                              | 0.004                         | 10.44           | 0.002           | Embodiment |
| E                       | E1 | -30           | 14.7                              | 0.003                         | 16.18           | 0.001           | Embodiment |
| F                       | F1 | -30           | 18.9                              | 0.001                         | 17.08           | 0.001           | Embodiment |
| G                       | G1 | -30           | 8.1                               | 0.006                         | 6.79            | 0.004           | Embodiment |
| H                       | H1 | -30           | 27.6                              | 0.001                         | 33.45           | 0.000           | Embodiment |
| I                       | I1 | -30           | 4.5                               | 0.004                         | 6.60            | 0.004           | Embodiment |
| J                       | J1 | -30           | 4.3                               | 0.005                         | 5.73            | 0.005           | Embodiment |
| K                       | K1 | -30           | 4.8                               | 0.005                         | 6.42            | 0.004           | Embodiment |

DP (I): a dew point temperature (° C.) of when a continuous annealing is performed

Amorphous: a thickness of an Si-based amorphous oxide layer

Oxide: a thickness of an Fe, Mn, and Cr oxide layer

TABLE 6

| Hot-Formed Member       |                |                |                           |               |                                   |                            |              |              |                      |                                |            |  |
|-------------------------|----------------|----------------|---------------------------|---------------|-----------------------------------|----------------------------|--------------|--------------|----------------------|--------------------------------|------------|--|
| Cold-Rolled Steel Plate | Classification | DP (II)<br>(□) | Tensile Strength<br>(MPa) | Surface Grade | Thickness of<br>Amorphous<br>(nm) | Thickness of Oxide<br>(μm) | Equation (4) | Equation (5) | Corrosion-resistance | Range of spot-weldability (kA) | Note       |  |
| D1                      | D1-1           | -10            | 1564                      | 2.8           | 52.4                              | 1.46                       | 68.85        | 1.57         | ○                    | 1.8                            | Embodiment |  |
| E1                      | E1-1           | -10            | 1506                      | 1.8           | 158.2                             | 1.85                       | 172.95       | 1.17         | ○                    | 1.6                            | Embodiment |  |
| F1                      | F1-1           | -10            | 1529                      | 1.50          | 194.6                             | 1.34                       | 184.20       | 1.13         | ○                    | 1.6                            | Embodiment |  |
| G1                      | G1-1           | -10            | 1535                      | 3.5           | 45.1                              | 2.65                       | 31.87        | 2.09         | ○                    | 2.2                            | Embodiment |  |
| H1                      | H1-1           | -10            | 1487                      | 1.5           | 351.2                             | 1.30                       | 387.61       | 0.72         | ○                    | 1.4                            | Embodiment |  |
| I1                      | I1-1           | -10            | 1495                      | 3.8           | 41.6                              | 2.45                       | 30.72        | 2.13         | ○                    | 2.2                            | Embodiment |  |
| J1                      | J1-1           | -10            | 1474                      | 3.7           | 38.7                              | 2.87                       | 24.46        | 2.34         | ○                    | 2.4                            | Embodiment |  |
| K1                      | K1-1           | -10            | 1513                      | 3.4           | 28.1                              | 2.49                       | 29.81        | 2.17         | ○                    | 2.4                            | Embodiment |  |

DP (II): a dew point temperature (° C.) of heat treatment

Amorphous: a thickness of an Si-based amorphous oxide layer

Oxide: a thickness of an Fe, Mn, and Cr oxide layer

## 19

As indicated in table 6, embodiments D1-1 to K1-1 satisfied the alloy composition and the manufacturing conditions of the exemplary embodiment, and accordingly, excellent corrosion-resistance and spot-weldability were secured.

While exemplary embodiments have been shown and described above, the scope of the present disclosure is not limited thereto, and it will be apparent to those skilled in the art that modifications and variations could be made without departing from the scope of the present invention as defined by the appended claims.

The invention claimed is:

1. A cold-rolled steel plate for hot-forming, having excellent corrosion-resistance and spot-weldability, comprising: C: 0.1 to 0.4%, Si: 0.5 to 2.0%, Mn: 0.01 to 4.0%, Al: 0.001 to 0.4%, P: 0.001 to 0.05%, S: 0.0001 to 0.02%, Cr: 0.5% or higher and less than 3.0%, N: 0.001 to 0.02%, and a balance of Fe and inevitable impurities by weight %,

wherein the cold-rolled steel plate satisfies equation (1) below:

$$1.4 \leq 0.4 * \text{Cr} + \text{Si} \leq 3.2$$

equation (1):

## 20

where each element symbol is a value of a content of each element measured by weight %; wherein an Si-based amorphous oxide layer having a thickness of 1 nm to 100 nm is continuously or discontinuously formed on a surface of the cold-rolled steel plate; and

wherein an Fe, Mn, and Cr oxide layer is formed to a thickness of 2.5  $\mu\text{m}$  or less on the Si-based amorphous oxide layer.

2. The cold-rolled steel plate of claim 1, wherein the cold-rolled steel plate further includes one or more selected from a) one or more selected from Ti, Nb, Zr, and V: 0.001 to 0.4% by weight %, and b) B: 0.0001 to 0.01% by weight %.

3. The cold-rolled steel plate of claim 1, wherein the cold-rolled steel plate further includes one or more selected from c) one or more of Mo and W: 0.001 to 1.0% by weight %, d) a sum of contents of Cu and Ni: 0.005 to 2.0% by weight %, and e) one or more of Sb and Sn: 0.001 to 1.0% by weight %.

4. The cold-rolled steel plate of claim 1, wherein a microstructure of the cold-rolled steel plate includes ferrite and cementite.

\* \* \* \* \*